

## 1

3,591,512

## CORROSION INHIBITOR

Morton W. Leeds, Murray Hill, N.J., assignor to Air Reduction Company, Incorporated, New York, N.Y.  
No Drawing. Filed Dec. 31, 1968, Ser. No. 788,997  
Int. Cl. C23g 1/06

U.S. CL. 252—148

3 Claims

## ABSTRACT OF THE DISCLOSURE

Aqueous acid solutions are inhibited against corrosion of metals, especially ferrous metals, by incorporation of a corrosion-inhibiting system composed of a combination of an acetylenic carbinol and a saturated heterocyclic nitrogen compound mixture derived from gilsonite.

This invention relates to the inhibition of metal corrosion in acidic solutions and is more particularly concerned with inhibited aqueous acid solutions suitable for the treatment of metals.

Metal cleaning baths and pickling baths generally comprise aqueous solutions of inorganic acids such as sulfuric acid, hydrochloric acid, and phosphoric acid, and are useful in the cleaning and treatment of iron, zinc, ferrous alloys, and the like.

In the use of aqueous acidic baths to treat metals, additives or inhibitors in the baths are desirable to prevent or inhibit corrosion or erosion of the metal surfaces. Similarly, in the field of oil-well acidizing, it is necessary to use inhibitors in order to prevent corrosion of the oil-well equipment by the aqueous acid solutions employed. Various other industrial operations also involve contact between an aqueous acidic solution and a metal, and an inhibitor must be used in order to minimize corrosion and/or consumption of the metal by such contact.

If no corrosion inhibitor is present when the aqueous acidic solution comes into contact with the metal, excessive metal loss, production of undesirable metal surface properties, excessive consumption or loss of acid, and like adverse results will be experienced. Many different types of inhibitors have been proposed, but there has been a continuing search for corrosion inhibitors which can be used effectively in small concentrations, and which are economical to produce, since the use of inhibitors is a necessary expense and it is economically prudent to keep this expense at a minimum while, at the same time, realizing the desired inhibition of metallic corrosion or consumption. The need is also for corrosion inhibitors which are effective at high temperatures, e.g. 200° F. and above, such as are encountered in various operations involving acidic solutions, particularly oil-well acidizing where higher and higher temperatures are encountered as the well extends further into the earth.

While various corrosion-inhibiting agents have been proposed, all of such agents are not of equal effectiveness and of the many hundreds of agents which have been contemplated, only a few are sufficiently active to be commercially attractive. This is particularly true in the case of high-temperature operations. Some inhibitors which have been proposed are reasonably effective at low and moderate temperatures, but fail completely when high temperatures are encountered.

There has, therefore, been a continuing search for more effective inhibitors, or for ways of making a given inhibitor more effective. This search has involved the discovery of combinations of inhibitors which act together to provide an inhibitor system. However, many of these systems involve relatively expensive components so that, while they may be relatively effective in their corrosion-inhibiting activity, there are disadvantages from an eco-

## 2

nomic standpoint, particularly if they have to be used in substantial quantities in order to bring about the desired corrosion-inhibiting activity. Similarly, many of these systems are ineffective at elevated temperatures. In particular, there is a need for a corrosion-inhibiting system comprising a plurality of components wherein relatively inexpensive compounds of poor corrosion-inhibiting action can be catalyzed or "potentiated" by the other component or components of the system so that the combination has a high corrosion-inhibiting activity even at elevated temperatures.

It is accordingly an object of this invention to provide a novel corrosion-inhibiting system involving a combination of agents which is highly effective from the standpoint of corrosion-inhibiting activity and which is, at the same time, commercially attractive.

It is a further object of this invention to provide a novel corrosion-inhibiting system comprising a combination of agents wherein one agent has a strong potentiating or catalyzing action upon the other agent so that the corrosion-inhibiting effectiveness of the combination is greater than the additive action of the components of the combination.

It is another object of the invention to provide a corrosion-inhibiting system of the character indicated which is effective at high temperatures.

In accordance with this invention, it has been discovered that the above and other objects can be achieved by the provision of a corrosion-inhibiting system comprising a combination of an acetylenic carbinol of the formula

30 R—CHOH—C≡CH, wherein R is a lower alkyl radical, i.e. containing up to 7 carbon atoms, which may form a straight chain or a branched chain, and a saturated heterocyclic nitrogen compound mixture derived from gilsonite. While any of the acetylenic carbinols falling within the 35 above formula are suitable, 1-hexyn-3-ol, wherein R=3, and 4-ethyl-1-octyn-3-ol, wherein R=7, have been found to be particularly suitable. The saturated nitrogen compound mixture is obtained by the hydrogenation of the unsaturated heterocyclic nitrogen compound mixture directly derived from gilsonite which generally can have a distillation range of about 350° F. to about 700° F., but most suitably there are employed fractions "cut" from this overall range by fractional distillation and hydrogenated, as will be described below. Hydrogenation does 40 not appreciably change the distillation range of the mixtures. A hydrogenated mixture or "fraction" of gilsonite-derived heterocyclic nitrogen compounds having a distillation range generally lying between about 350° F. and 600° F. is preferably used. All temperatures are at 760 45 mm. While the mixture is referred to as being composed of "saturated" heterocyclic nitrogen compounds, it will be understood that minor amounts of the corresponding unsaturated compounds may be present as a result of incomplete hydrogenation. The ratio between the acetylenic 50 alcohol component and the saturated heterocyclic nitrogen compound mixture component of the corrosion-inhibiting system may vary, but the best results are obtained with weight ratios ranging between 1:10 and 10:1, preferably 1:5 and 5:1, and most suitably between 1:2 and 55 2:1.

The acetylenic alcohol-heterocyclic nitrogen compound mixture inhibition system of this invention is useful, in general, in the inhibition of corrosion of metal surfaces in contact with aqueous mineral acid solution, such as hydrochloric acid, sulfuric acid, and phosphoric acid, for example in the acidizing of oil wells, in electrolytic cleaning baths, and electrolytic refining of metals, as well as in metal cleaning and pickling baths. The use of the acetylenic alcohol-nitrogen compound mixture inhibitor system 60 of this invention for corrosion inhibition of metals in aqueous mineral acid solutions is advantageous in that the acetylenic alcohol-nitrogen compound mixture system can

be employed as a corrosion inhibitor over a wide and useful concentration range. A further advantage of this inhibitor system is that it may be used at elevated temperatures to provide good corrosion inhibition, even when in relatively low concentration.

The most effective amount of the corrosion-inhibiting system to be used in accordance with this invention can vary, depending upon local operation conditions. Thus, the temperature and other characteristics of the acid corrosive system may have a bearing upon the amount of inhibitor to be used. The higher the temperature and/or the higher the acid concentration, the greater is the amount of corrosion inhibitor required to give optimum results. In general, however, it has been found that a concentration of the corrosion-inhibiting system of the invention between 0.01 and 2%, preferably between 0.01% and 1.2%, by weight of the aqueous acidic solution is an effective corrosion-inhibiting concentration, although higher concentrations can be used when conditions make them desirable, with a concentration between 0.05% to 0.75% by weight being of most general use, at elevated temperatures, e.g. in the neighborhood of 200° F. The acidic solution can be dilute or concentrated and can be of any of the concentrations used in treating metals, e.g. ferrous metals, or for operations involving contact of acidic solutions with such metals, e.g. oil-well acidizing, and the like, for example 5 to 80%. In most operations of the character indicated, acid concentrations of 10-15% by weight are employed, and non-oxidizing inorganic acids are used. However, it is not intended to limit the invention to any specific use of acidic solutions or with respect to any specific metal or acid.

Gilsonite is a natural asphalt-like substance found in the Uinta Basin in Utah and, when coked by application of heat, which results in the distillation of volatile materials, produces an oily distillate as the temperature is increased. This distillate has an overall boiling range of about 350 up to about 900, although most of it boils below 700, and when it is refined by treatment with sulfuric acid, produces mixtures of heterocyclic nitrogen compounds. These mixtures are generally fractionally distilled to provide a series of fractions. Such fractions derived from the Gilsonite distillate are sold by the American Gilsonite Company of Salt Lake City, Utah. One of these fractions, sold commercially under the trade designation GN-200 is catalytically hydrogenated, and this hydrogenated fraction, which is sold under the trade designation GN-300, is suitably employed as one of the components of the system of this invention to provide the hydrogenated heterocyclic nitrogen compound content. The following are typical distillation ranges in ° F. (ASTM D-158):

## GN-200

| Vol. percent: | ° F. |
|---------------|------|
| Start         | 361  |
| 10            | 448  |
| 30            | 492  |
| 50            | 514  |
| 70            | 532  |
| 90            | 550  |
| End           | 579  |

## GN-300

| Vol. percent: | ° F. |
|---------------|------|
| Start         | 351  |
| 10            | 444  |
| 30            | 479  |
| 50            | 503  |
| 70            | 526  |
| 90            | 552  |
| End           | 592  |

The exact composition of these fractions is not fully known, but it is believed that the principal components are as follows: GN-200: alkylated pyrroles, indoles, pyridines, and quinolines; GN-300: primarily ring-saturated secondary amines, e.g. alkylated piperidines, quinolines,

pyrrolidines and indolines, the balance of the mixture being made up of unsaturated heterocyclic, alkylated, tertiary amines such as methyl-substituted pyrrole, indole, pyridine, and quinoline.

The method used to determine the inhibiting properties of the system of the invention employs test specimens or coupons. To prepare the coupons, they are wiped with acetone to remove any residual oils or grease, and pickled for one minute in 10% hydrochloric acid to eliminate any scale and surface film. After pickling, the coupons are dipped in sodium bicarbonate solution, rinsed well in tap water, rinsed in distilled water, and finally dried with acetone. The clean and dry specimens are then weighed to the nearest 0.1 mg. In carrying out the evaluation, hydrochloric acid of 15% by weight concentration is used in order to duplicate oil-well acidizing conditions. The inhibitor system is added to 4 oz. test bottles, 100 ml. of the acid then added to each bottle; and the mixture shaken vigorously. The bottles are suspended in a constant-temperature bath consisting of a bell jar filled with ethylene glycol and equipped with a stirrer. The temperature is regulated to maintain the samples at 200±2° F. The bottles are placed in the bath ½ hour before the test coupons are added to insure temperature equilibrium. The weighed coupons, in duplicate, are then supported on glass hooks in the test bottles and the bottles are covered with watch glasses during the testing period of 16 hours. At the end of the testing period, the bottles are removed from the bath, the coupons withdrawn, rinsed with water, sodium bicarbonate solution, distilled water, and dried in acetone, then weighed to measure weight loss. Corrosion-inhibiting properties are conveniently expressed as percent inhibition, using the following formula:

Percent inhibition

$$= \frac{\text{Wt. loss of blank} - \text{wt. loss of test coupon}}{\text{wt. loss of blank}} \times 100$$

When the acid concentration and temperature are such that the blank would be completely consumed by the acid in the absence of an inhibitor, the foregoing formula can be expressed as:

Percent inhibition

$$= \frac{\text{Original wt. test coupon} - \text{wt. loss of test coupon}}{\text{original wt. test coupon}} \times 100$$

The following experiments will serve to illustrate the effectiveness of the corrosion-inhibiting system of this invention under severe corrosion conditions encountered in practical application:

## EXAMPLE

Using the testing procedure described above, and employing test coupons of mild steel 1 in. x 2 in. x 1/16 in. in size, samples comprising 1-hexyn-3-ol or 4-ethyl-1-octyn-3-ol in combination with a mixture of saturated heterocyclic nitrogen compounds as represented by a commercial fraction of the character described above, in 1:1 weight ratio, were added to 15% hydrochloric acid, each component of the combination being added in the amount of 0.12% by weight of the acid, and the combination evaluated for corrosion-inhibiting activity. At the same time a blank test, using the same acid but without any inhibitor, was made. The following results were obtained:

| Inhibitor:                          | Percent inhibition, 16 hrs. |
|-------------------------------------|-----------------------------|
| 1-hexyn-3-ol+GN-300 (0.24%)         | 99+                         |
| 4-ethyl-1-octyn-3-ol+GN-300 (0.24%) | 99+                         |
| None                                | —                           |

These tests show the positive action of the combination of an acetylenic carbinol and a mixture of saturated heterocyclic nitrogen compounds in accordance with this

invention in inhibiting metal corrosion in an acid solution of high concentration at an elevated temperature only slightly below the boiling point of water, over a prolonged period of time, the components of the system being relatively inexpensive chemicals in the corrosion-inhibiting field. Corresponding results are obtained when other acetylenic carbinols and other saturated nitrogen compound mixtures within the definitions set forth above are employed in forming the inhibiting system of this invention.

The coupons used in the foregoing experiments were cut from a  $\frac{1}{16}$  in. sheet of a mild steel having the following typical analysis: 0.15% max. carbon, 0.30-0.60% manganese, 0.04% phosphorus, 0.05% sulfur, the balance iron.

It will be understood that various changes and modifications may be made in the operations described in the foregoing without departing from the scope of the invention as defined in the appended claims. It is intended, therefore, that all matter contained in the above description of the invention shall be interpreted as illustrative only and not as limitative.

I claim:

1. A metal corrosion-inhibitor system for use with aqueous mineral acids which consists essentially of an acetylenic carbinol of the formula  $R-CHOHC\equiv CH$ , wherein  $R$  is a lower alkyl group, and a saturated heterocyclic nitrogen compound mixture derived from gilsonite and distilling within the range of about 350° F. and about

700° F. at 760 mm. Hg, said acetylenic carbinol and said mixture being in the relative weight ratios of 1:10 and 10:1.

2. A corrosion-inhibited mineral acid consisting essentially of an aqueous solution of the mineral acid and a small but effective amount of a corrosion-inhibiting system consisting essentially of an acetylenic carbinol of the formula  $R-CHOHC\equiv CH$ , wherein  $R$  is a lower alkyl group, and a saturated heterocyclic nitrogen compound mixture derived from gilsonite and distilling within the range of about 350° F. and about 700° F. at 760 mm. Hg, said acetylenic carbinol and said mixture being in the relative weight ratios of 1:10 and 10:1.

3. A corrosion-inhibited acid as defined in claim 2, wherein said corrosion-inhibiting system is present in the amount of 0.01% to 2% by weight.

#### References Cited

##### UNITED STATES PATENTS

|    |           |         |                       |          |
|----|-----------|---------|-----------------------|----------|
| 20 | 3,107,221 | 10/1963 | Harrison et al. ----- | 252—148  |
|    | 3,249,548 | 5/1966  | Herman et al. -----   | 252—148X |
|    | 3,404,094 | 10/1968 | Keeney -----          | 252—148  |
|    | 3,432,527 | 3/1969  | Malec et al. -----    | 252—392  |

MAYER WEINBLATT, Primary Examiner

U.S. CL. X.R.

21—2.5; 252—8.5, 136, 390, 392, 394